



US010549893B2

(12) **United States Patent**  
**Peck**

(10) **Patent No.:** **US 10,549,893 B2**  
(45) **Date of Patent:** **\*Feb. 4, 2020**

(54) **METHOD FOR CONTROLLING OXYGEN INGRESS IN CAP CLOSURE**

(71) Applicant: **G3 Enterprises, Inc.**, Modesto, CA (US)

(72) Inventor: **James Peck**, Modesto, CA (US)

(73) Assignee: **G3 Enterprises, Inc.**, Modesto, CA (US)

(\*) Notice: Subject to any disclaimer, the term of this patent is extended or adjusted under 35 U.S.C. 154(b) by 167 days.

This patent is subject to a terminal disclaimer.

(21) Appl. No.: **14/082,065**

(22) Filed: **Nov. 15, 2013**

(65) **Prior Publication Data**

US 2014/0076841 A1 Mar. 20, 2014

**Related U.S. Application Data**

(63) Continuation-in-part of application No. 13/725,983, filed on Dec. 21, 2012.

(Continued)

(51) **Int. Cl.**

**B65D 51/00** (2006.01)

**B65D 51/16** (2006.01)

(Continued)

(52) **U.S. Cl.**

CPC ..... **B65D 51/1605** (2013.01); **B65B 3/02** (2013.01); **B65D 41/045** (2013.01)

(58) **Field of Classification Search**

CPC ..... B65D 51/24; B65D 51/244; B65D 51/20; B65D 53/04; B32B 27/00; B32B 27/06; B32B 27/08

(Continued)

(56)

**References Cited**

U.S. PATENT DOCUMENTS

5,673,809 A 10/1997 Ohmi et al.  
5,829,608 A 11/1998 Clerget

(Continued)

FOREIGN PATENT DOCUMENTS

CN 101891031 A 11/2010  
FR 1226696 A 7/1960

(Continued)

OTHER PUBLICATIONS

NPL: Evergreen, The barrier performance of common plastic film, [www.evergreen-packaging.com](http://www.evergreen-packaging.com).\*

(Continued)

*Primary Examiner* — Ernesto A Grano

(74) *Attorney, Agent, or Firm* — Goodwin Procter LLP

(57)

**ABSTRACT**

A system and method for controlling oxygen ingress in cap closures is disclosed. According to one embodiment, an apparatus includes a cap and a cap liner. The cap liner includes a first diffusive layer and a semi-diffusive layer. A first side of the semi-diffusive layer is adjacent to the first diffusive layer, where the semi-diffusive layer has a lower oxygen transmission rate than that of the first diffusive layer. The cap liner further includes a second diffusive layer, where a first side of the second diffusive layer is adjacent to a second side of the semi-diffusive layer, and the semi-diffusive layer has a lower oxygen transmission rate than that of the second diffusive layer. The oxygen transmission rate of the cap liner is controlled by varying a thickness of the semi-diffusive layer.

**6 Claims, 15 Drawing Sheets**



**Related U.S. Application Data**

(60) Provisional application No. 61/579,611, filed on Dec. 22, 2011.

**(51) Int. Cl.**

*B65D 41/04* (2006.01)  
*B65B 3/02* (2006.01)

**(58) Field of Classification Search**

USPC ..... 215/341, 232, 364, 347, 228, 201, 203  
See application file for complete search history.

**(56) References Cited**

## U.S. PATENT DOCUMENTS

6,082,566 A \* 7/2000 Yousif et al. .... 215/232  
6,139,931 A \* 10/2000 Finkelstein et al. .... 428/36.6  
6,866,926 B1 \* 3/2005 Smelko et al. .... 428/319.1  
6,902,075 B2 \* 6/2005 O'Brien et al. .... 215/232  
7,798,359 B1 \* 9/2010 Marsella .... 220/359.3  
8,703,265 B2 \* 4/2014 Thorstensen-Woll et al. ....  
428/66.4  
2002/0012808 A1 \* 1/2002 Ishizaki et al. .... 428/516  
2002/0162818 A1 11/2002 Williams  
2004/0191445 A1 9/2004 Baranowski et al.  
2007/0007229 A1 \* 1/2007 Yousif .... 215/232  
2007/0298273 A1 \* 12/2007 Thies .... B32B 27/32  
428/516  
2009/0026166 A1 1/2009 Druitt  
2009/0123766 A1 5/2009 Peck

2009/0208729 A1 \* 8/2009 Allegaert et al. .... 428/319.9  
2010/0213193 A1 \* 8/2010 Helmlinger et al. .... 220/200  
2012/0067842 A1 3/2012 Keller  
2012/0111758 A1 \* 5/2012 Lo ..... 206/524.6  
2012/0118764 A1 \* 5/2012 Valus et al. .... 206/213.1

## FOREIGN PATENT DOCUMENTS

FR 1249847 A 1/1961  
FR 1279992 A 12/1961  
FR 2821064 A1 8/2002  
WO WO-2004070410 A1 8/2004  
WO WO-2006113000 A2 10/2006  
WO WO-2006113000 A3 10/2006

## OTHER PUBLICATIONS

NPL: Mieke Buntinx, Gert Willems, Griet Knockaert, Dimitri Adons, Jan Yperman, Robert Carleer and Roos Peeters; Evaluation of the Thickness and Oxygen Transmission Rate before and after Thermoforming Mono- and Multi-layer Sheets into Trays with Variable Depth; polymers ISSN 2073-4360; www.mdpi.com/journal/polymers.\*

Supplementary European Search report dated Aug. 25, 2017 in corresponding EP Application No. EP15744075, filed Jul. 27, 2016, Inventor(s) Torrison, Miriam, et al.

International Search Report dated Feb. 22, 2013 in corresponding PCT Application No. PCT/US2012/71444 filed Dec. 21, 2012, inventor, Peck, James.

\* cited by examiner



Figure 1



Figure 2



Figure 3



Figure 4(a)

Figure 4(b)



Figure 5



Figure 6(a)

Figure 6(b)

Figure 6(c)



Figure 7



Figure 8



Figure 9



Figure 10



Figure 11



Figure 12



Figure 13



Figure 14(b)

Figure 14(a)

OTR



Figure 15

## METHOD FOR CONTROLLING OXYGEN INGRESS IN CAP CLOSURE

The present application is a continuation-in-part of U.S. patent application Ser. No. 13/725,983, entitled "Method for Controlling Oxygen Ingress in Cap Closure", filed on Dec. 21, 2012, which claims the benefit of and priority to U.S. Provisional Application Ser. No. 61/579,611, entitled "Method for Controlling Oxygen Ingress in Aluminum Cap Closure", filed on Dec. 22, 2011, the disclosures of which are incorporated by reference in their entirety, for all purposes, herein.

### FIELD

The present application relates in general to methods controlling oxygen ingress in cap closures. In particular, the present application is directed to methods controlling oxygen transmission in cap liners.

### BACKGROUND

Most wines exhibit a chemical oxygen demand required for the proper development of flavors, mouthfeel and aromas. This development is termed "wine maturation". A cap closure that allows the correct amount of oxygen into a wine bottle will promote wine maturation at an ideal rate, otherwise referred to as aging. If a cap closure has no oxygen barrier, too much oxygen will cause the wine to oxidize rapidly and shorten its shelf life. It is commonly known within the wine industry that white wines are much more sensitive to oxygen while red wines are generally more tolerant of exposure to oxygen. It is generally accepted that the proper amount of oxygen entering the wine at a proper rate through the closure will have a beneficial effect on wine quality.

The traditional closure for wine is the bark of the *Quercus Suber*, commonly known as cork oak. The oxygen transmission rate (OTR) of a premium natural cork is considered by many winemakers to be the gold standard. Premium wines using such corks are normally stored inverted or laid on their side. Storing wine in this manner reduces the OTR by keeping the cork wet, thus enhancing its sealing capabilities.

In the current wine industry, aluminum screw-cap closures have become a popular alternative to cork closures due to their low cost and predictable performance. The crucial sealing performance of a cap is controlled to a large extent by its liner component. Cap liners are required to seal sufficiently to prevent the beverage from leaking out of the package. They are also crucial for controlling the transmission of oxygen from the air outside the package into the product while retaining volatile flavor molecules in the beverage. Liner types have traditionally been chosen by cap manufacturers (e.g., G3), with a focus on ease of use, performance and price. It is not commonly known how to precisely select a combination of materials and their thicknesses to obtain a desired OTR over a range of OTRs.

There are two major cut-disk cap liner technologies that dominate the cap liner industry (e.g., cap liners manufactured by MEYER SEALS), those containing SARANEX<sup>TM</sup> (a polyvinylidene chloride (PVDC)/polyethylene (PE) laminate that provides barrier protection) as an oxygen barrier and those utilizing a combination of SARANEX<sup>TM</sup> with either tin or aluminum foil as the oxygen barrier. The OTR of these two cap liner designs are uniform at their respective values, the foil-SARANEX<sup>TM</sup> being much lower than the SARANEX<sup>TM</sup> alone.

The SARANEX<sup>TM</sup> layer is typically thin, ranging from 1.0 to 2.0 mils. SARANEX<sup>TM</sup> itself is normally a five layer laminate, the outermost layers being low-density polyethylene (LDPE) film with adhesive layers (e.g., ethylene-vinyl acetate (EVA)) or a similar tie-layer polymer between the LDPE and the PVDC. The PVDC is the oxygen barrier component of SARANEX. Most of the total thickness of the SARANEX<sup>TM</sup> film is due to the layers of LDPE and adhesive. The LDPE and the adhesive layers have very high OTR relative to PVDC and metal foils. The SARANEX<sup>TM</sup> cap liner is considered by some to allow too much oxygen into the wine, leading to a decreased shelf-life. The foil-SARANEX<sup>TM</sup> cap liner is known to allow almost no oxygen into the wine bottle, which can cause anaerobic conditions resulting in reduced or sulfidic aromas. Therefore, some in the wine industry believe that foil-SARANEX<sup>TM</sup> liners allow in too little oxygen. OTR tests of inverted natural premium Flor grade corks using the OX-TRAN (a system for oxygen transmission rate testing) system from MOCON (a provider 10 for oxygen permeation detection instruments) determined that their OTR values were between those of SARANEX<sup>TM</sup> and foil-SARANEX<sup>TM</sup> cap liners.

There are currently no commercial cap liners for wine screw caps that provide OTR values close to that of a premium inverted natural bark cork. One prior attempt to create this range of OTR values was made by producing liners using different thickness of ethylene vinyl alcohol (EVOH) in place of the SARANEX<sup>TM</sup> barrier. However, the OTR of three thicknesses of EVOH were virtually identical to each other and very close to the OTR of a SARANEX<sup>TM</sup> cap liner. Another prior attempt was made using perforated metalized polymer, which resulted in unacceptable variability in OTR values.

Another prior attempt to achieve the desired OTR 35 included applying various perforation schemes through tin foil and then using the perforated foil to create a laminate liner similar to a foil-SARANEX<sup>TM</sup> liner. However, this produced neither the desired control of OTR, nor an OTR close to that of a wine package finished with a premium 40 natural bark cork. The perforations in the foil, which may be known as the primary barrier, did not control the OTR. The OTR values of this configuration were similar to that of a foil-SARANEX<sup>TM</sup> liner without perforations in the tin foil.

### SUMMARY

A system and method for controlling oxygen ingress in cap closures is disclosed. According to one embodiment, an apparatus includes a cap and a cap liner. The cap liner includes a first diffusive layer and a semi-diffusive layer. A first side of the semi-diffusive layer is adjacent to the first diffusive layer, where the semi-diffusive layer has a lower oxygen transmission rate than that of the first diffusive layer. The cap liner further includes a second diffusive layer, where 50 a first side of the second diffusive layer is adjacent to a second side of the semi-diffusive layer, and the semi-diffusive layer has a lower oxygen transmission rate than that of the second diffusive layer. The oxygen transmission rate of the cap liner is controlled by varying a thickness of 55 the semi-diffusive layer.

The above and other preferred features, including various novel details of implementation and combination of events, will now be more particularly described with reference to the accompanying figures and pointed out in the claims. It 60 will be understood that the particular systems and methods described herein are shown by way of illustration only and not as limitations. As will be understood by those skilled in

the art, the principles and features described herein may be employed in various and numerous embodiments without departing from the scope of the present disclosure.

#### BRIEF DESCRIPTION OF THE DRAWINGS

The accompanying figures, which are included as part of the present specification, illustrate the presently preferred embodiments of the present disclosure and together with the general description given above and the detailed description of the preferred embodiments given below serve to explain and teach the principles described herein.

FIG. 1 illustrates an exploded view of components in a cap liner, according to one embodiment.

FIG. 2 illustrates an exploded view of components in a cap liner, according to one embodiment.

FIG. 3 illustrates an exploded view of components in a cap liner, according to one embodiment.

FIG. 4(a) illustrates an exemplary plot of a factor effect in a model for OTR control, according to one embodiment.

FIG. 4(b) illustrates another exemplary plot of a factor effect in a model for OTR control, according to one embodiment.

FIG. 5 illustrates an exploded view of components in a cap liner, according to one embodiment.

FIG. 6(a) illustrates an exemplary plot of the effect of the thickness of highly diffusive layers on OTR, according to one embodiment.

FIG. 6(b) illustrates another exemplary plot of the effect of the thickness of highly diffusive layers on OTR, according to one embodiment.

FIG. 6(c) illustrates an exemplary plot of the effect of different materials on OTR, according to one embodiment.

FIG. 7 illustrates an exploded view of components in a cap liner, according to one embodiment.

FIG. 8 illustrates an exploded view of components in a cap liner, according to one embodiment.

FIG. 9 illustrates an exploded view of components in a cap liner, according to one embodiment.

FIG. 10 illustrates an exploded view of components in a cap liner, according to one embodiment.

FIG. 11 illustrates a cross-sectional view of components in a cap liner, according to one embodiment.

FIG. 12 illustrates a flow chart of an exemplary process for controlling oxygen ingress in cap closures, according to one embodiment.

FIG. 13 illustrates an exploded view of components in a cap liner, according to one embodiment.

FIG. 14(a) illustrates a plot of an exemplary model for OTR control, according to one embodiment.

FIG. 14(b) illustrates another plot of an exemplary model for OTR control, according to one embodiment.

FIG. 15 illustrates another flow chart of an exemplary process for controlling oxygen ingress in a cap closure, according to one embodiment.

It should be noted that the figures are not necessarily drawn to scale and are only intended to facilitate the description of the various embodiments described herein. The figures do not describe every aspect of the teachings described herein and do not limit the scope of the claims.

#### DETAILED DESCRIPTION

A system and method for controlling oxygen ingress in cap closures is disclosed. According to one embodiment, an apparatus includes a cap and a cap liner. The cap liner includes a first diffusive layer and a semi-diffusive layer. A

first side of the semi-diffusive layer is adjacent to the first diffusive layer, where the semi-diffusive layer has a lower oxygen transmission rate than that of the first diffusive layer. The cap liner further includes a second diffusive layer, where a first side of the second diffusive layer is adjacent to a second side of the semi-diffusive layer, and the semi-diffusive layer has a lower oxygen transmission rate than that of the second diffusive layer. The oxygen transmission rate of the cap liner is controlled by varying a thickness of the semi-diffusive layer.

According to one embodiment, the present disclosure describes a cap liner design that delivers OTR including a range of OTR between the OTR of SARANEXT™ and foil-SARANEXT™ liners, and also an extended range of higher OTR. This allows the creation of custom OTRs for cap closures. The present cap liner design provides the OTR of a premium bark cork, according to one embodiment. The present cap liner design provides the OTR of a synthetic cork, according to another embodiment.

FIG. 1 illustrates an exploded view of components in a cap liner, according to one embodiment. The cap liner 100 includes a first highly diffusive layer 104, a secondary oxygen barrier 103, a second highly diffusive layer 102, a primary oxygen barrier 101, and a backing layer 107. The first side of the first highly diffusive layer 104 is adjacent to the first side of the secondary oxygen barrier 103. The second side of the first highly diffusive layer 104 contacts the lip-sealing surface 105 of a bottle 106. The second side of the secondary oxygen barrier 103 is adjacent to the first side of the second highly diffusive layer 102. The second side of the second highly diffusive layer 102 is adjacent to a first side of the primary oxygen barrier 101. The second side of the primary oxygen barrier 101 is adjacent to one side of the backing layer 107. The backing layer 107 may include materials made of LDPE foam, paper card and other types of backing material known in the art. The secondary oxygen barrier 103 may include films made of PVDC, Polyester (PET), EVOH, metalized PET (by vacuum deposition), metalized LDPE, metalized ultra low density polyethylene (ULDPE), metalized linear low-density polyethylene (LLDPE), metalized high-density polyethylene (HDPE), a metalized layer or any oxygen barrier known in the art, according to one embodiment. The primary oxygen barrier 101 may include films made of tin foil, aluminum foil, PVDC, Polyester (PET), EVOH, metalized PET (by vacuum deposition), metalized LDPE, metalized ultra low density polyethylene (ULDPE), metalized linear low-density polyethylene (LLDPE), metalized high-density polyethylene (HDPE), a metalized layer or any oxygen barrier known in the art, according to one embodiment. In one embodiment, the primary oxygen barrier 101 is a better barrier to oxygen than the secondary oxygen barrier 103, i.e., the primary oxygen barrier 101 has a lower OTR than the secondary oxygen barrier 103 based on various factors, such as a thickness and a material type. The first highly diffusive layer 104 and the second highly diffusive layer 102 may include one or more types of highly diffusive polymers known in the art, according to one embodiment. The first highly diffusive layer 104 and the second highly diffusive layer 102 may include, but are not limited to very low density polyethylene (VLDPE), LDPE, EVA, HDPE, LLDPE, and ULDPE films according to one embodiment. The first highly diffusive layer 104 and the second highly diffusive layer 102 may include one or more types of highly diffusive polymers known in the art, according to one embodiment. The OTR of

the cap liner 100 is controlled by varying the thicknesses of the first highly diffusive layer 104 and the second highly diffusive layer 102.

FIG. 2 illustrates an exploded view of components in a cap liner, according to one embodiment. The cap liner 200 includes a highly diffusive layer 202, a primary oxygen barrier layer 201, and a backing layer 205. The first side of the primary oxygen barrier layer 201 is adjacent to one side of the backing layer 205. The second side of the primary oxygen barrier layer 201 is adjacent to one side of the highly diffusive layer 202. The other side of the highly diffusive layer 202 contacts the lip-sealing surface 203 of a bottle 204. The backing layer 205 may include materials made of LDPE foam, paper card and other types of backing material known in the art. The primary oxygen barrier 201 may include films made of tin foil, aluminum foil, PVDC, Polyester (PET), EVOH, metallized PET (by vacuum deposition), metallized LDPE, metallized ultra low density polyethylene (ULDPE), metallized linear low-density polyethylene (LLDPE), metallized high-density polyethylene (HDPE), a metallized layer or any oxygen barrier known in the art, according to one embodiment. The highly diffusive layer 202 may include VLDPE, LDPE, EVA, HDPE, LLDPE, and ULDPE films, according to one embodiment. The highly diffusive layer 202 may include one or more types of highly diffusive polymers known in the art, according to one embodiment. The OTR of the cap liner 200 is controlled by varying the thickness of the highly diffusive layer 202.

FIG. 3 illustrates an exploded view of components in a cap liner, according to one embodiment. The cap liner 300 includes a LDPE foam 301, a layer of metal foil 302, a first layer of highly diffusive materials ("B" layer) 303, a layer of PVDC 304 and a second layer of highly diffusive materials ("A" layer) 305. One side of the highly diffusive "A" layer 305 contacts the lip-sealing surface 306 of a bottle 307. The layer of PVDC 304 and the layer of metal foil 302 may be considered as oxygen barrier layers. The materials from the "A" layer 305 and the "B" layer 303 may include one or more types of highly diffusive polymers known in the art, according to one embodiment. The materials from the "A" layer 305 and the "B" layer 303 may include, but are not limited to VLDPE, LDPE, EVA, HDPE, LLDPE and ULDPE films, according to one embodiment. The thicknesses of the "A" layer 305 and the "B" layer 303 on either side of the layer of PVDC 304 are the OTR controlling factors. The control of oxygen ingress is exercised by varying the thickness of the "B" layer of highly diffusive materials 303 between the layer of metal foil 302 and the layer of PVDC 304, as well as the thickness of the "A" layer of highly diffusive materials 305 between the layer of PVDC 304 and the lip-sealing surface 306 of the bottle 307. The thicknesses of the "A" layer 305 and the "B" layer 303 on both sides of the secondary oxygen barrier layer of PVDC 304 are particularly important for targeting and controlling the desired OTR, including the diffusive layers that are a part of a SARANEX™ laminate. In a traditional cap liner, the highly diffusive layers on either side of the layer of PVDC are typically 0.5 to 3.5 mils thick. However, the thicknesses of the highly diffusive "A" layer 305 and the highly diffusive "B" layer 303 may vary from 1 to 10 mils thick, depending upon the target OTR, according to one embodiment. A mathematical model that defines how OTR values vary with changes in the thickness of the highly diffusive layers is developed, according to one embodiment. The mathematical model may be a prediction equation created using statistical modeling software (e.g., JMP (a statistical discovery software)) to determine how the thickness of the highly diffusive

layers control the OTR of the cap liner using the same layer of PVDC, according to one embodiment. The present system selects a combination and thicknesses of highly diffusive materials on both sides of an oxygen barrier layer to obtain a desired OTR over a range of OTR.

Referring to FIG. 4(a) and FIG. 4(b), the respective thicknesses of the "A" layer 305 and "B" layer 303 corresponding to the desired OTR are determined. The model's leverage plots in FIGS. 4(a) and 4(b) are used to determine the thicknesses of the "A" layer 305 and the "B" layer 303 to achieve the desired OTR. In particular, the plots show that the thickness of the "A" layer 305 between the layer of PVDC 304 and the bottle 307 has a greater effect on OTR than the thickness of the "B" layer 303 on the other side of the layer of PVDC 304 further away from the lip-sealing surface 306 of the bottle 307. According to one embodiment, the unit for OTR is cc O<sub>2</sub>/cap/day.

The path for the majority of the oxygen diffusion in an aluminum cap is through the liner's edge. Therefore, oxygen is entering the films in the liner through their edge, moves past the lip-sealing surface of the bottle, and then into the bottle. The diffusion of gases is proportional to the surface area of edge material exposed to air. The OTR increases with increasing thickness of the highly diffusive layers as more surface area is exposed to air.

The OTR of materials measured in the form of flat sheets is different from the OTR of the same material when inserted into an aluminum cap and secured on a bottle. The normal direction of gas diffusion in a flat sheet is perpendicular to the surface of the sheet. However, the OTR of a liner inside an aluminum cap is primarily controlled by gas diffusion that is perpendicular to the liner's edge.

According to one embodiment, the effect of different SARANEX™ films and the effect of different thicknesses of highly diffusive EVA adhesive films placed at two locations in the cap liner on OTR were evaluated. Referring to FIG. 5, the cap liner 500 includes a layer of LDPE foam 501, a first layer of EVA ("EVA1" layer) 502, a layer of tin foil 503, a second layer of EVA ("EVA2" layer) 504, and a layer ("C" layer) 505 of either SARANEX™ or LDPE film. One side of the "C" layer 505 contacts the lip-sealing surface 506 of a bottle 507. In a designed experiment, the effect on OTR of using three different SARANEX™ films or a 2 mil LDPE film for the "C" layer 505 were evaluated. The effect on OTR of the thickness of the "EVA1" layer 502 and the thickness of the "EVA2" layer 504 placed above and below the tin foil 503 respectively were also evaluated using three thicknesses. Table 1 below illustrates the various configurations for each sample in the experiment.

TABLE 1

| Sample | "EVA1" Layer           |                        | "EVA2" Layer           |                        |
|--------|------------------------|------------------------|------------------------|------------------------|
|        | Thickness (mil)<br>502 | Thickness (mil)<br>504 | Thickness (mil)<br>505 | Thickness (mil)<br>505 |
| 1A     | 7                      | 1                      | 2 mil LDPE             |                        |
| 1B     | 7                      | 1                      | 2 mil LDPE             |                        |
| 1C     | 7                      | 1                      | 2 mil LDPE             |                        |
| 2A     | 7                      | 1                      | SARANEX™ 3             |                        |
| 2B     | 7                      | 1                      | SARANEX™ 3             |                        |
| 2C     | 7                      | 1                      | SARANEX™ 3             |                        |
| 3A     | 1                      | 1                      | SARANEX™ 1             |                        |
| 3B     | 1                      | 1                      | SARANEX™ 1             |                        |
| 3C     | 1                      | 1                      | SARANEX™ 1             |                        |
| 4A     | 7                      | 7                      | SARANEX™ 1             |                        |
| 4B     | 7                      | 7                      | SARANEX™ 1             |                        |
| 4C     | 7                      | 7                      | SARANEX™ 1             |                        |
| 5A     | 1                      | 7                      | SARANEX™ 3             |                        |

TABLE 1-continued

| Sample | “EVA1” Layer Thickness (mil)<br>502 | “EVA2” Layer Thickness (mil)<br>504 | “C” Layer<br>505 |
|--------|-------------------------------------|-------------------------------------|------------------|
| 5B     | 1                                   | 7                                   | SARANEX™ 3       |
| 5C     | 1                                   | 7                                   | SARANEX™ 3       |
| 6A     | 7                                   | 7                                   | SARANEX™ 0       |
| 6B     | 7                                   | 7                                   | SARANEX™ 0       |
| 6C     | 7                                   | 7                                   | SARANEX™ 0       |
| 7A     | 1                                   | 1                                   | SARANEX™ 0       |
| 7B     | 1                                   | 1                                   | SARANEX™ 0       |
| 7C     | 1                                   | 1                                   | SARANEX™ 0       |
| 8A     | 1                                   | 7                                   | 2 mil LDPE       |
| 8B     | 1                                   | 7                                   | 2 mil LDPE       |
| 8C     | 1                                   | 7                                   | 2 mil LDPE       |
| 9A     | 4                                   | 4                                   | SARANEX™ 0       |
| 9B     | 4                                   | 4                                   | SARANEX™ 0       |
| 9C     | 4                                   | 4                                   | SARANEX™ 0       |
| 10A    | 4                                   | 4                                   | SARANEX™ 1       |
| 10B    | 4                                   | 4                                   | SARANEX™ 1       |
| 10C    | 4                                   | 4                                   | SARANEX™ 1       |

FIGS. 6(a)-6(c) illustrate the effect of different SARANEX™ films and the effect of different thicknesses of highly diffusive EVA adhesive films placed at two locations in the cap liner on OTR according to the exemplary cap liner in FIG. 5. Referring to the plot in FIG. 6(c), there is little difference between the OTR when three different types of SARANEX™ are used. However, when LDPE is used for the “C” layer 505, the OTR of the cap liner 500 is significantly higher than the OTR when SARANEX™ is used. The plot in FIG. 6(b) shows that there is essentially no effect on OTR when the thickness of the highly diffusive “EVA1” layer 502 is varied. The plot in FIG. 6(a) shows that there is a significant effect on OTR when the thickness of the highly diffusive “EVA2” layer 504 is varied. This indicates that oxygen is bypassing the barrier of the tin foil 503 when the thickness of the “EVA2” layer 504 is increased at this location, i.e., on the side of the tin foil 503 nearer to the lip-sealing surface 506 of the bottle 507.

According to one embodiment, the effects of different thicknesses of highly diffusive films between a PVDC layer and the bottle finish on OTR are evaluated. Referring to FIG. 7, the cap liner 700 includes 50 mil thickness of LDPE foam 701, 1 mil of EVA adhesive 702, 1 mil of tin foil 703, 2 mil of highly diffusive film (“B” layer) 704, a layer of PVDC 705 and a layer of highly diffusive film (“A” layer) 706. The “A” layer of highly diffusive film 706 is between the layer of PVDC 705 and the lip-sealing surface 707 of the bottle 708. The effect of the thickness of the highly diffusive “A” layer 706 on OTR is illustrated using a thickness of 3, 7 and 11 mils of EVA and LDPE as the highly diffusive “A” layer 706. Table 2 below shows that OTR increases with increment in the thickness of the “A” layer 706. The cap liner 700 precisely controls oxygen transmission by varying the thickness of the highly diffusive materials between the PVDC 705 and the lip-sealing surface 707 of the bottle 708.

TABLE 2

| “B” Layer Thickness (mil)<br>704 | “A” Layer Thickness (mil)<br>706 | OTR     |
|----------------------------------|----------------------------------|---------|
| 2                                | 3                                | 0.00023 |
| 2                                | 7                                | 0.00048 |
| 2                                | 11                               | 0.00064 |

According to one embodiment, the effects of different thickness of highly diffusive films between a tin foil layer

and the bottle finish on OTR are evaluated. Referring to FIG. 8, the cap liner 800 includes a 50 mil thickness of LDPE foam 801, 1 mil of EVA adhesive 802, 1 mil of tin foil 803 and a layer of highly diffusive film (“A” layer) 804. The “A” layer of highly diffusive film 804 is between the tin foil 803 and the lip-sealing surface 805 of the bottle 806. The effect of the thickness of the “A” layer 804 on OTR is tested using a thickness of 3, 7 and 11 mils of EVA and LDPE as the highly diffusive “A” layer 804 that is configured to be in contact with the sealing surface 805 of the bottle 806. Table 3 below shows that OTR increases with increment in the thickness of the “A” layer 804. The cap liner 800 precisely controls oxygen transmission by varying the thickness of the highly diffusive materials between the tin foil 803 and the lip-sealing surface 805 of the bottle 806.

TABLE 3

| “A” Layer Thickness (mil)<br>804 | OTR     |
|----------------------------------|---------|
| 3                                | 0.00014 |
| 7                                | 0.00023 |
| 11                               | 0.00041 |

According to one embodiment, the effect of different thickness of highly diffusive films between semi-permeable Polyester (PET) film and the bottle finish on OTR are evaluated. Referring to FIG. 9, the cap liner 900 includes a 50 mil thickness of LDPE foam 901, 1.5 mil of EVA adhesive 902, 0.35 mil of aluminum foil 903, a layer of 1.5 mil of LDPE film (“B” layer) 904, 0.5 mil of semi-diffusive PET film 905 and a layer of highly diffusive film (“A” layer) 908. The “A” layer includes 1 mil of EVA adhesive 906 and 1 mil of LDPE film 907. The “A” layer 908 is between the semi-permeable PET film 905 and the lip-sealing surface 909 of the bottle 910. The effect of a combination of the EVA adhesive 906 and the LDPE film 907 on OTR is evaluated using a thickness of LDPE film 907 of 4, 8 and 12 mils, producing the “A” layer 908 of 5, 9 and 13 mils of highly diffusive films. Table 4 below shows that OTR increases with increment in the thickness of the “A” layer 908 that includes the EVA adhesive 906 and the LDPE film 907. The cap liner 900 precisely controls oxygen transmission by varying the thickness of the highly diffusive materials between the semi-diffusive PET film 905 and the lip-sealing surface 909 of the bottle 910.

TABLE 4

| “B” Layer Thickness (mil)<br>904 | “A” Layer Thickness (mil)<br>908 | OTR    |
|----------------------------------|----------------------------------|--------|
| 1.5                              | 5                                | 0.0011 |
| 1.5                              | 9                                | 0.0013 |
| 1.5                              | 13                               | 0.0014 |

According to one embodiment, the effect of different thickness of highly diffusive films between a vacuum deposition metalized layer and the bottle finish on OTR are evaluated. Referring to FIG. 10, the cap liner 1000 includes a 50 mil thickness of LDPE foam 1001, 1.5 mil of EVA adhesive 1002, 0.35 mil of aluminum metalized PET film 1003 and a layer of highly diffusive film (“A” layer) 1006. The “A” layer 1006 includes 1 mil of EVA adhesive film 1004 and a LDPE film 1005. The “A” layer 1006 is between the vacuum deposition aluminum metalized PET film 1003

and the lip-sealing surface 1007 of the bottle 1008. The effect of a combination of the EVA adhesive 1004 and the LDPE film 1005 on OTR is evaluated using a thickness of LDPE film 1005 of 4, 8 and 12 mils, producing the "A" layer 1006 of 5, 9 and 13 mils of highly diffusive film. Table 5 below shows that OTR increases with increment in the thickness of the "A" layer 1006 that includes the EVA adhesive 1004 and the LDPE film 1005. The cap liner 1000 precisely controls oxygen transmission by varying the thickness of the highly diffusive materials between the aluminum metalized PET film 1003 and the lip-sealing surface 1007 of the bottle 1008.

TABLE 5

| "A" Layer<br>Thickness (mil) | OTR    |
|------------------------------|--------|
| 1006                         |        |
| 5                            | 0.0008 |
| 9                            | 0.0010 |
| 13                           | 0.0012 |

According to one embodiment, the effect of different thickness of highly diffusive films between a vacuum deposition metalized layer and the bottle finish on OTR are evaluated. Referring to FIG. 11, the cap liner 1100 includes a 50 mil thickness of LDPE foam 1101, 1.5 mil of EVA adhesive 1102, 0.35 mil of aluminum metalized LDPE film 1103, and a layer of highly diffusive film ("A" layer) 1106. The "A" layer 1106 includes 1 mil of EVA adhesive film 1104 and a LDPE film 1105. The "A" layer 1106 is between the vacuum deposition aluminum metalized LDPE film 1103 and the lip-sealing surface 1107 of the bottle 1108. The effect of a combination of the EVA adhesive 1104 and the LDPE film 1105 on OTR is evaluated using a thickness of LDPE film 1105 of 4, 8 and 12 mils, producing the "A" layer 1106 of 5.5, 9.5 and 13.5 mils of highly diffusive film. Table 6 below shows that OTR increases with increment in the thickness of the "A" layer 1106 that includes the EVA adhesive 1104 and the LDPE film 1105. The cap liner precisely controls oxygen transmission by varying the thickness of the highly diffusive materials between the aluminum metalized LDPE film 1103 and the lip-sealing surface 1107 of the bottle 1108.

TABLE 6

| "A" Layer<br>Thickness (mil) | OTR    |
|------------------------------|--------|
| 1106                         |        |
| 5.5                          | 0.0011 |
| 9.5                          | 0.0013 |
| 13.5                         | 0.0014 |

According to one embodiment, the present method is used for plastic cap liners. As there is additional diffusion of oxygen through the shell of the plastic cap, adjustments to the model may be necessary.

FIG. 12 illustrates a flow chart of an exemplary process for controlling oxygen ingress in a cap closure, according to one embodiment. At 1200, a backing material for the liner is selected. The backing material may include, but is not limited to, expanded LDPE foam and any backing material typically used by one with ordinary skill in the art, according to one embodiment. At 1201, a primary oxygen barrier is selected. The primary oxygen barrier may include, but is not limited to, films made of tin foil, aluminum foil, PVDC,

Polyester (PET), EVOH, metalized PET (by vacuum deposition), metalized LDPE, metalized ultra low density polyethylene (ULDPE), metalized linear low-density polyethylene (LLDPE), metalized high-density polyethylene (HDPE), a metalized layer or any oxygen barrier known in the art, according to one embodiment. At 1202, the first side of the primary oxygen barrier is placed adjacent to the backing material. At 1203, a first diffusive layer is selected. The first diffusive layer may include one or more types of highly diffusive polymers known in the art, according to one embodiment. The first diffusive layer may include, but is not limited to, VLDPE, low-density polyethylene (LDPE), EVA, high-density polyethylene (HDPE), linear low-density polyethylene (LLDPE) and ultra low density polyethylene (ULDPE) films, according to one embodiment. At 1204, the first side of the first diffusive layer is placed adjacent to the second side of the primary oxygen barrier. At 1205, a secondary oxygen barrier layer is selected. The secondary oxygen barrier may include films made of PVDC, Polyester (PET), EVOH, metalized PET (by vacuum deposition), metalized LDPE, metalized ultra low density polyethylene (ULDPE), metalized linear low-density polyethylene (LLDPE), metalized high-density polyethylene (HDPE), a metalized layer or any oxygen barrier known in the art, according to one embodiment. At 1206, the first side of the secondary barrier layer is placed adjacent to the second side of the first diffusive layer. At 1207, the second diffusive layer is selected. The second diffusive layer may include one or more types of highly diffusive polymers known in the art, according to one embodiment. The second diffusive layer may include, but are not limited to, VLDPE, LDPE, EVA, high-density polyethylene (HDPE), linear low-density polyethylene (LLDPE) and ultra low density polyethylene (ULDPE) films, according to one embodiment. At 1208, the first side of the second diffusive layer is placed adjacent to the second side of the secondary oxygen barrier. The backing material, the primary oxygen barrier, the first diffusive layer, the secondary oxygen barrier, and the second diffusive layer form part of a cap liner in a cap closure, according to one embodiment. After the materials are selected for a part of the cap liner, a model that predicts how OTR varies with the thicknesses of the first and second diffusive layers is developed at 1209. After the model is developed, a graph of the dependent variable OTR versus changes in the thicknesses of the first and the second diffusive layers is created at 1210. The desired OTR is selected at 1211. At 1212, the thicknesses of the first and second diffusive layers corresponding to the desired OTR are selected from the graph.

According to one embodiment, the present cap liner design delivers a range of OTR between that of a typical cap liner employing tin-SARANEX™ as an oxygen barrier and a cap liner employing SARANEX™ as an oxygen barrier. This allows the creation of a cap closure having the OTR of a premium quality natural cork.

According to one embodiment, the present cap liner design includes a first highly diffusive backing layer, a semi-diffusive oxygen barrier layer, and a second highly diffusive layer. The semi-diffusive oxygen barrier layer has an OTR higher than SARANEX™ but lower than that of LDPE. It is noted that the materials selected for a highly diffusive layer, a semi-diffusive oxygen barrier layer, and a primary/secondary oxygen barrier are arranged in the order of decreasing OTR. It is further noted that the materials LDPE, PET, SARANEX™, and Tin-SARANEX™ (or aluminum-SARANEX™) are arranged in the order of decreasing OTR. The first highly diffusive backing layer may include any highly diffusive material used for the construc-

## 11

tion of cap liners, such as a polymer foam, a paper card, and a combination thereof. The first highly diffusive backing layer is adjacent to a first side of the semi-diffusive oxygen barrier layer. A first side of the second highly diffusive layer is adjacent to a second side of the semi-diffusive oxygen barrier layer. The second side of the second highly diffusive layer may contact a lip-sealing surface of a bottle. The material of the second highly diffusive layer may include any highly diffusive polymer film material, but is not limited to VLDPE, LDPE, EVA, high-density polyethylene (HDPE), linear low-density polyethylene (LLDPE) and ultra low density polyethylene (ULDPE) films, according to one embodiment. The OTR of the present cap liner is controlled by varying the thickness of the semi-diffusive oxygen barrier layer. Varying the thickness of the semi-diffusive oxygen barrier layer provides a greater effect on the OTR than varying the thickness of the second highly diffusive layer that contacts a lip-sealing surface of a bottle. In particular, the OTR of the present cap liner design increases as the thickness of the semi-diffusive oxygen barrier layer decreases, i.e., the OTR of the present cap liner design increases as the inverse of the thickness of the semi-diffusive oxygen barrier layer increases. The use of a semi-diffusive layer allows the production of a custom OTR for cap closures having higher OTR than cap closures that include an oxygen barrier layer made of various materials such as a metal foil, SARANEX™ EVOH, and any other high oxygen barrier materials. The present cap liner design provides an OTR similar to that of a synthetic (polymer foam) cork, according to one embodiment.

FIG. 13 illustrates an exploded view of components in a cap liner, according to one embodiment. The cap liner 1300 includes a first highly diffusive layer 1301, a layer of semi-diffusive film 1302, and a second highly diffusive layer 1303. One side of the second highly diffusive layer 1303 contacts the lip-sealing surface 1304 of a bottle 1305. The materials for the first highly diffusive layer 1301 may include, but are not limited to, an expanded polymer foam that includes VLDPE, LDPE, HDPE, ULDPE, LLDPE, polypropylene (PP), and EVA. The material for the second highly diffusive layer 1303 may include, but are not limited to, one or more films with high oxygen transmission rates, such as VLDPE, LDPE, HDPE, ULDPE, LLDPE, PP, and EVA.

According to one embodiment, the OTR of the cap liner 1300 is controlled by the thickness of the semi-diffusive film 1302. The material for the semi-diffusive film 1302 may include, but is not limited to PET and polyethylene terephthalate glycol-modified (PETG). The control of oxygen ingress is exercised by varying the thickness of the semi-diffusive film 1302 between the first highly diffusive layer 1301 and the second highly diffusive layer 1303. The thickness of the semi-diffusive film 1302 has a greater effect on targeting and controlling the OTR of the cap liner 1300 than the thicknesses of the second highly diffusive layer 1303 and the first highly diffusive layer 1301.

FIG. 14(a) and FIG. 14(b) illustrate plots of exemplary models for OTR control. The respective thickness of the second highly diffusive layer 1303 and the layer of semi-diffusive film 1302 corresponding to the desired OTR are determined. The model's leverage plots in FIG. 14(a) and FIG. 14(b) are used to determine the thicknesses of the second highly diffusive layer 1303 and the layer of semi-diffusive film 1302 to achieve a desired OTR. FIG. 14(b) illustrates that OTR increases linearly with the inverse of the thickness of the semi-diffusive film 1302. However FIG. 14(a) illustrates that the thickness of the second highly

## 12

diffusive layer 1303 has negligible effect on OTR. The thickness of the semi-diffusive film 1302 that is required to achieve a desired OTR can be determined from the plot in FIG. 14(b).

FIG. 15 illustrates another flow chart of an exemplary process for controlling oxygen ingress in a cap closure, according to one embodiment. At 1501, a first diffusive layer is selected. The first diffusive layer may include one or more types of highly diffusive cap liner backing materials known in the art, according to one embodiment. The first diffusive layer may include, but is not limited to, VLDPE, LDPE, HDPE, ULDPE, LLDPE, PP, and EVA foams, according to one embodiment. At 1502, a semi-diffusive layer is selected. At 1503, the first side of the semi-diffusive layer is placed adjacent to the first diffusive layer. At 1504, a second diffusive layer is selected. The second diffusive layer may include one or more types of highly diffusive polymers known in the art, according to one embodiment. The second diffusive layer may include, but are not limited to VLDPE, LDPE, EVA, EAA, High-density Polyethylene (HDPE), Linear Low-density Polyethylene (LLDPE) and Ultra Low Density Polyethylene (ULDPE) films, according to one embodiment. At 1505, the first side of the second diffusive layer is placed adjacent to the second side of the semi-diffusive layer. The second side of the second diffusive layer may be in contact with a lip-sealing surface of a bottle. The first diffusive layer, the semi-diffusive layer, and the second diffusive layer form part of a cap liner in a cap closure, according to one embodiment. After the materials are selected for a part of the cap liner, a model that predicts how OTR varies with the thickness of the semi-diffusive layer is developed at 1506. After the model is developed, a graph of the dependent variable OTR versus changes in the thicknesses of the semi-diffusive layer is plotted at 1507. The desired OTR is selected at 1508. At 1509, the thicknesses of the semi-diffusive layer corresponding to the desired OTR are selected from the graph.

The above example embodiments have been described hereinabove to illustrate possible embodiments for controlling oxygen transmission rate of cap liners. Various modifications to and departures from the disclosed example embodiments will occur to those having ordinary skill in the art. The subject matter that is intended to be within the spirit of this disclosure is set forth in the following claims.

I claim:

1. An apparatus, comprising:  
a cap; and  
a cap liner,  
wherein the cap liner includes a first diffusive layer,  
wherein the first diffusive layer is 2 mil and comprises  
one or more of SARANEX™ and LDPE,  
wherein the cap liner includes a 1 mil metalized layer,  
wherein a first oxygen transmission rate of the metalized  
layer is lower than a second oxygen transmission rate  
of the first diffusive layer,  
wherein the cap liner includes an adhesive layer of 1 mil  
to 7 mil between the first diffusive layer and the  
metalized layer,  
wherein the cap liner includes a second diffusive layer,  
wherein the first oxygen transmission rate of the metalized  
layer is lower than a third oxygen transmission rate of  
the second diffusive layer,  
wherein a thickness of the first diffusive layer is variable  
to control a total oxygen transmission rate of the cap  
liner such that the cap liner has a total oxygen trans-  
mission rate increase as the thickness of the first  
diffusive layer increases.

2. The apparatus of claim 1, wherein the total oxygen transmission rate of the cap liner increases linearly with an inverse of the thickness of the first diffusive layer.

3. The apparatus of claim 1, wherein the second diffusive layer comprises an expanded foam of one or more of very low density polyethylene (VLDPE), polypropylene (PP), low-density polyethylene (LDPE), ethylene-vinyl acetate (EVA), high-density polyethylene (HDPE), linear low-density polyethylene (LLDPE), and ultra low density polyethylene (ULDPE). <sup>5</sup>

4. The apparatus of claim 1, wherein the first diffusive layer further comprises one or more of very low density polyethylene (VLDPE), polypropylene (PP), ethylene-vinyl acetate (EVA), high-density polyethylene (HDPE), linear low-density polyethylene (LLDPE) and ultra low density <sup>10</sup> polyethylene (ULDPE) film.

5. The apparatus of claim 1, wherein the first diffusive layer is configured to contact a lip-sealing surface of a bottle.

6. The apparatus of claim 1, wherein the total oxygen transmission rate matches that of a synthetic cork. <sup>15</sup> <sup>20</sup>

\* \* \* \* \*